

## 1

3,725,051

### METHOD OF PURIFYING LOW-CARBON FERROCHROME

Cecil George Chadwick, Lewiston, N.Y., assignor to Union Carbide Corporation, New York, N.Y.  
No Drawing. Filed Oct. 14, 1970, Ser. No. 80,811  
Int. Cl. C22c 1/06, 39/14

U.S. Cl. 75—130.5

1 Claim

#### ABSTRACT OF THE DISCLOSURE

Method for lowering the nitrogen, carbon and oxygen content of ferrochromium alloy by heating the alloy under vacuum.

This invention relates to the removal of nitrogen, carbon and oxygen from low carbon ferrochromium alloys. More particularly this invention is directed to the purification of ferrochromium alloys by vacuum furnacing.

Low carbon ferrochromium alloy, intended for use as an alloy addition agent to steel is produced by reacting molten chrome ore and lime with ferrochrome silicon alloy in an electric furnace to produce molten ferrochromium alloy which is thereafter cast into slabs or ingots to provide ferrochromium alloy in massive form. The massive alloy is subsequently crushed to suitable industrial size such as 2 inches and finer. The ferrochromium alloy in this form is dense, homogeneous and easily handled. Such alloy ordinarily contains in addition to iron and chromium, from about 0.10 to 0.13% nitrogen, 0.022 to 0.05% carbon and 0.05 to 0.12% oxygen. Such nitrogen, carbon and oxygen contents are generally undesirably high for additions to be used in the making of high performance alloy steels.

It is therefore an object of the present invention to provide ferrochromium alloy having very low nitrogen, carbon and oxygen contents.

Other objects will be apparent from the following description and claims.

A method in accordance with the present invention comprises heating ferrochromium metal under vacuum at elevated temperatures to provide ferrochromium containing not more than about 0.02% nitrogen, 0.01% carbon and 0.07% oxygen.

In the practice of the present invention, ferrochromium alloy obtained by the solidification of molten ferrochromium for example containing 71 to 74% Cr, 25 to 28% Fe, 0.10 to 0.13% N<sub>2</sub>, 0.022 to 0.05% C and 0.05 to 0.12% O<sub>2</sub>, is heated under vacuum at temperatures in the range of 1300 to 1400° C. at pressures of from 60 to 500 microns. Suitable furnacing times are from 10 to 40 hours, preferably from 30 to 40 hours.

As a result of the foregoing treatment, the nitrogen content of the ferrochromium can be reduced to less than 0.02%, the carbon can be reduced to less than 0.01% and the oxygen can be reduced to less than

## 2

0.07%. This result, i.e. the concurrent removal of nitrogen, carbon and oxygen, is surprising and leads to the production of a highly desirable material. For example, ferrochromium alloy treated in accordance with the present invention can be readily utilized in vacuum melting operations to produce high performance alloy steels.

The following examples will further illustrate the present invention.

#### EXAMPLE I

Chromium ore and lime were charged to an electric furnace. The foregoing constituents were then reacted with ferrochrome silicon to produce molten ferrochromium alloy. The molten ferrochromium alloy was teemed and cast into slabs. The massive ferrochromium alloy was subsequently crushed to obtain lumps of alloy about 2 inches in size. Approximately 15.0 lbs. of the lump ferrochromium containing about 71% Cr, 26% Fe was placed in a vacuum furnace and heated at about 1385° C. for various times up to forty hours at an absolute pressure of about 100 microns. Analysis of the alloy before and after the vacuum furnacing treatments is shown in Table I.

TABLE I

|                       | Initial | After 10 hours | After 20 hours | After 40 hours |
|-----------------------|---------|----------------|----------------|----------------|
| Percent carbon.....   | 0.04    | 0.01           | 0.007          | 0.008          |
| Percent nitrogen..... | 0.10    | 0.037          | 0.016          | 0.012          |
| Percent oxygen.....   | 0.12    | 0.08           | 0.09           | 0.07           |

From the foregoing data it can be seen that after a vacuum furnacing treatment of forty hours the nitrogen content of the alloy was reduced to about one tenth of its initial value, the oxygen content was reduced to about one-half of its initial value, and the carbon content was reduced to one-fifth of its initial value.

What is claimed is:

1. A process for lowering the nitrogen, carbon and oxygen content of particulated low carbon ferrochromium alloy which comprises heating the particulated ferrochromium at a temperature in the range of about 1300 to 1400° C. under vacuum of about 500 to 100 microns for a period of time from about 20 to 40 hours whereby a product containing not more than 0.02% nitrogen, 0.01% carbon and 0.07% oxygen is obtained.

#### References Cited

##### UNITED STATES PATENTS

|           |        |          |       |            |
|-----------|--------|----------|-------|------------|
| 2,541,153 | 2/1951 | Chadwick | ----- | 148—13.1 X |
| 2,624,671 | 1/1953 | Binder   | ----- | 75—126     |
| 3,523,021 | 8/1970 | Khitrik  | ----- | 75—130.5 X |

55 L. DEWAYNE RUTLEDGE, Primary Examiner

J. E. LEGRU, Assistant Examiner